# EUROPEAN PATENT SPECIFICATION

(11) **EP 0 513 523 B1**
(45) Date of publication and mention of the grant of the patent: **29.07.1998**
(21) Application number: 92106005.9
(22) Date of filing: 07.04.1992
(51) Int. Cl.: B22D 17/00, C22C 1/00

(54) **Die casting process for producing high mechanical performance components via injection of a semiliquid metal alloy**
Druckgussverfahren zur Herstellung von Teilen mit hoher mechanischer Leistungsfähigkeit aus thixotropem Metall
Procédé pour le moulage par injection d'articles avec un excellent fonctionnement mécanique, d'un métal à l'état de mélange liquide-solide

(30) Priority: 19.04.1991 IT TO910299
(43) Date of publication of application: 19.11.1992
(73) Proprietor: MAGNETI MARELLI S.p.A., 20145 Milano (IT)
(72) Inventor: Moschini, Renzo, I-60019 Senigallia (IT)
(74) Representative: Cerbaro, Elena

(56) References cited:
- GB-A- 2 112 676
- VDI ZEITSCHRIFT vol. 133, no. 3, March 1991, DUESSELDORF WOLFGANG SCHNEIDER: 'Formgiessverfahren für innovative Aluminiumgussteile' p. 127-128, 131-133
- MéMOIRES ET ETUDES SCIENTIFIQUES DE LA REVUE DE MéTALLURGIE vol. 80, no. 7/8,
- August 1983, PARIS pages 355 - 365; C. MILLIERE ET AL.: 'Structure, propriétés et mise en forme des alliages brassés à l'état semi-solide (suite)'
- METALLURGICAL TRANSACTIONS B vol. 22B, no. 3, June 1991, WARRENDALE, PA, US pages 269 - 293; MERTON C. FLEMINGS: 'Behavior of Metal Alloys in the Semisolid State'

## Description

The present invention relates to a die casting process for producing internal combustion engine components from a light alloy, in particular, aluminium alloy to which ceramic particles are added.

Italian Patent n.1.119.287 filed on 20 June, 1979, and entitled: "Process and device for preparing a metal alloy mixture comprising a solid and liquid phase", the content of which is incorporated herein purely by way of reference as required, relates to a static mixer consisting of a cylindrical runner housing a series of helical blades, for casting and partially solidifying a metal alloy as it is fed through the mixer, while at the same time mixing the newly formed solid phase with the remaining liquid phase. This produces, at the output of the mixer, a relatively low-viscosity solid/liquid mixture in which the solid phase of the alloy is uniformly suspended in the liquid alloy.

For the solid/liquid mixture to remain stable long enough for ladling and casting, it must be produced under steady fluid dynamic conditions, with accurate, rapid control of the physical and dynamic parameters involved in the casting process (temperature, alloy cooling rate, speed through the mixer, etc.). For this purpose, the present Applicant has perfected a semiliquid casting process as described in Italian Patent Application n.67 627-A/89, filed on 25.07.1989, and entitled: "Continuous semiliquid casting process and furnace", the content of which is incorporated herein purely by way of reference as required. According to the above process, the static mixer is connected to a pressurized tiltable reverberatory furnace, for casting under steady conditions, and is equipped with a barometric column enabling it to be refilled without interrupting or affecting steady flow of the casting.

Metal alloys produced using semiliquid casting processes as described above or other similar processes, as described, for example, in "VDI Zeitschrift" vol. 133 no. 3, March 1991, p. 127-128, 131-133, or "Memoires et etudes scientifique de la revue de metallurgie" (p. 355-365) are said to be "rheocast", and present particularly good microstructural characteristics. Rheocast light alloys, in fact, have recently be found to present a globular as opposed to a traditional dendritic microstructure, thus resulting in improved fluid dynamic characteristics (temperatures within the solidification range). Despite the above advantages, however, known semiliquid casting processes have yet to be applied to the manufacture of internal combustion engine components, which, for cost reasons, are normally die cast. A major drawback of die casting is the formation of blowholes in the casting, resulting from the turbulence produced by the high speed at which the liquid alloy is injected. Another drawback is inevitable shrinkage of the casting as it solidifies, and which is proportional to the temperature at which the alloy is injected (which, for liquid aluminium alloy is usually 700°C). Though cheap to produce, the poor quality of current die cast components therefore makes the use of finer quality alloys unfeasible.

Apart from the fact that they cannot be used for die casting, the above consideration also applies to various recently marketed alloys reinforced with ceramic particles to give 20 to 30% greater mechanical strength as compared with nonreinforced alloys of the same type. In fact, even assuming the reinforcing particles (which, being ceramic, melt at a much higher temperature than light alloy) could be maintained evenly dispersed in the molten alloy, e.g. by stirring it, the problem still remains of preventing the particles from separating from the alloy and accumulating in one part of the casting by force of gravity and, more especially, the dynamic thrust exerted on the particles as the molten alloy is fed, in this case, under turbulent flow conditions, through the gate.

It is an object of the present invention to provide a process enabling low-cost manufacture of metal alloy die castings with substantially no defects, and using fine quality metal alloys, possibly also containing uniformly dispersed ceramic reinforcing elements.

According to the present invention, there is provided a process for producing die castings, in particular, light alloy internal combustion engine components, as claimed in claim 1.

According to the present invention, there is also provided a process for die casting aluminium alloy, as claimed in claim 6.

A non-limiting embodiment of the present invention will be described by way of example with reference to the accompanying drawings, in which:
Fig.s 1 and 2 show schematic views of the various stages in the process according to the present invention;
Fig.s 3 and 4 show respective microphotographs of the same metal alloy before and after certain stages in the process according to the present invention.

With reference to Fig.s 1 and 2, pigs 1 of a metal alloy, in the example shown, light aluminium-based casting alloy UNI 3600 (UNI coding) are first melted normally in a known pot furnace 2. According to a preferred embodiment of the present invention, the initial alloy is A356, a casting alloy produced and marketed by ALCAN of San Diego (CA) U.S.A., which presents a nominal matrix of 93% Al and 7% Si in which is dispersed uniformly a ceramic phase consisting, in this case, of SiC (silicon carbide) particles. These, with a volumetric percentage of 20% for a given composition, provide for a roughly 30% improvement in the mechanical characteristics of the alloy and, in particular, a roughly 35% reduction in thermal expansion, which is thus similar to that of steel. In this case, furnace 2 is equipped with a known mechanical mixer 3 (or other similar known means not shown for the sake of simplicity) for maintaining the SiC particles uniformly dispersed in the molten alloy.

Once the initial alloy is fully liquefied (except for any suspended SiC particles, which melt at a much higher temperature than the alloy), the resulting liquid phase 4 (possibly also containing solid SiC particles) is fed into a pressurized rocking furnace 6 as described in Italian Patent Application n. 67627-A/89, filed by the present Applicant on 25.07.1989, and the content of which is incorporated herein purely by way of reference as required; which furnace 6 is connected to a known static mixer 7 as described in Italian Patent n. 1.119.287 filed on 20 June, 1979, and the content of which is also incorporated herein purely by way of reference as required.

Liquid phase 4 is then cast as described in the above patents, the mixer 7 being cooled so as to separate from liquid phase 4, as it is fed through mixer 7, a solid phase (not shown) which gradually increases as the alloy is cooled through mixer 7, and which is mixed uniformly with liquid phase 4 to produce a temporary stable solid-liquid suspension 8 at the output of mixer 7. During this stage, any solid SiC particles in the original alloy are also mixed continually with liquid phase 4 in mixer 7 to form an integral part of suspension 8 with no risk of the particles being segregated.

Suspension 8 is cast, for example, in an ingot mold 10 to produce an ingot 11 consisting of the original metal alloy, and possibly also containing dispersed SiC particles, but which, due to being cast in semiliquid form, presents an entirely different crystal structure. In pig 1 form, for example, a UNI 3600 alloy presents a dendritic structure as shown in Fig.3, whereas, when rheocast (i.e. cast in semiliquid form through mixer 7) and solidified, the same alloy presents a globular structure as shown in Fig.4.

Ingot 11 is then divided, e.g. cut mechanically using known means, such as a circular saw, into a number of smaller ingots 12, each, including the feedhead and channels, roughly equal to the weight of the component for casting, and which are fed, in stainless steel containers 13 (Fig.2), into an electric resistance furnace 14, preferably specially designed and equipped with automatic robot handling devices 15, where they are heated (for 50-60 minutes) to a temperature within the solidification range of the initial metal alloy. The rheocast globular-structure alloy of ingots 12 (with or without uniformly dispersed SiC particles) thus assumes a semiliquid state having, in the example shown, a liquid phase percentage of roughly 50% by volume, i.e. substantially the same as at the semiliquid casting stage through mixer 7.

When cast through mixer 7, however, the semiliquid alloy, by virtue of mixer 7, presents at most a viscosity of a few P, whereas, in ingot 12 form, by appropriately selecting the chemical composition and the heating temperature within the solidification range of the initial alloy (roughly 580°C for aluminium alloys), the same semiliquid alloy, but with a globular structure and heated to said temperature within the solidification range of the initial alloy, has been found to present substantially pseudoplastic rheologic characteristics and a viscosity at rest of about 10⁷ P. At the output of furnace 14, the alloy of ingots 12 therefore presents a pasty, pudding-like consistency preventing the segregation of any solid ceramic particles, which thus remain uniformly dispersed in the alloy, and enabling ingots 12 to maintain their shape.

Ingots 12 processed as described above are then fed one at a time on to a known die casting machine 18 (not described in detail) fitted with the same molds normally used for liquid alloys, with the exception of the gates, the thickness of which is increased from 0.8:1 mm to 2:2.5 mm to assist throughput of the semiliquid alloy. The semiliquid ingot 12 is fed into a known injection chamber 20 on machine 18, where it is subjected by a piston 21 to a predetermined mechanical pressure, equal to that usually employed for die casting liquid alloys, e.g. 650 Kg/cm², and injected into a mold 22 where the alloy solidifies to produce a finished casting 25 consisting, for example, of an internal combustion engine component, such as an injection manifold.

By virtue of the semiliquid form in which it is fed into chamber 20, however, the alloy, as compared with a liquid alloy of the same composition, presents a much higher viscosity and, therefore, a very low Reynolds number, thus enabling injection under laminar flow conditions, as opposed to turbulent flow conditions typical of known liquid alloy die casting processes. The high viscosity at rest combined with laminar-flow injection of the alloy provides, on the one hand, for preventing the inclusion of air bubbles and the formation of blowholes in the finished casting, and, on the other, for preventing the segregation of any solid ceramic particles contained in the semiliquid alloy fed on to machine 18, which particles therefore remain uniformly dispersed both in the semiliquid alloy injected into mold 22 and in the finished casting 25. Nor is the injection stage in any way hampered by the high viscosity at rest of the semiliquid globular alloy, which, being pseudoplastic, reduces its viscosity, when subjected to pressure by piston 21, to a P value of a few tens, compatible with low energy consumption of machine 18.

## Claims

1. A process for producing die castings, in particular, light alloy internal combustion engine components, comprising stages consisting in:
- melting a metal alloy until it is fully liquid;
- casting said metal alloy in semiliquid form;
- solidifying said metal alloy in semiliquid form into rheocast ingots wherein the metal alloy presents a globular micrographic structure;
- dividing said rheocast ingots into a number of ingots of predetermined weight, by mechanically cutting said rheocast ingots;
- heating said cut ingots to a temperature within the solidification range of said metal alloy, to convert the globular-structure metal alloy into paste form;
- feeding said ingots, one at a time, into the injection chamber of a die casting machine; and
- injecting said globular-structure alloy, heated to said temperature within the solidification range of the alloy, into a mold;
- characterized by the fact that, in combination:
(a)- said casting of the metal alloy in semiliquid form is carried out by feeding the melted metal alloy, as it, solidifies and under laminar flow conditions, through a static mixer for mixing the liquid alloy uniformly with a solid phase, which separates from the liquid alloy to produce a temporary stable solid-liquid suspension at the output of the mixer;
(b)- said cutting of the rheocast ingot is carried out in such a manner that each cut ingot of predetermined weight presents the same weight as the component for casting;
(c)- said heating of said cut ingots to a temperature within the solidification range of said metal alloy is carried out putting each cut ingot inside a respective stainless steel container and heating the ingot and the container into a preheating furnace.

2. A process as claimed in Claim 1, characterized by the fact that said temperature within the solidification range of said alloy and the chemical composition of said alloy are so selected that said globular-structure alloy heated to a temperature within the solidification range of the alloy assumes substantially pseudoplastic rheologic characteristics and a viscosity at rest of about 10⁷ P.

3. A process as claimed in Claim 2, characterized by the fact that, during said injection stage, said metal alloy comprises a solid phase and a liquid phase; said solid phase being equal to at least 50% by volume.

4. A process as claimed in any one of the foregoing Claims, characterized by the fact that said melting stage consists in melting pigs of aluminium alloy containing a predetermined percentage of a finely dispersed ceramic material phase; and is conducted in a pot furnace equipped with mixing means.

5. A process as claimed in Claim 4, characterized by the fact that said ceramic phase consists of silicon carbide particles.

6. A process for die casting aluminium alloy, consisting in heating an ingot, produced by casting said alloy in semiliquid form to produce a globular micrographic structure of the alloy, to a temperature within the solidification range of the alloy and such as to reduce the alloy to a highly viscous, semiliquid form; and in subsequently exerting mechanical pressure on the ingot; characterized by the fact that it employs molds having a gate the thickness of which is about 2 ö 2.5 mm; and by the fact that it employs an aluminium alloy containing a uniformly dispersed ceramic material phase.

## Patentansprüche

1. Verfahren zum Herstellen von Spritzgußteilen, insbesondere Verbrennungsmotor-Komponenten aus Leichtmetall, mit Verfahrensschritten, die bestehen in:
- dem Schmelzen einer Metallegierung bis sie vollkommen verflüssigt ist;
- dem Gießen dieser Metallegierung im halbflüssigen Zustand;
- dem Verfestigen dieser Metallegierung im halbflüssigen Zustand in Rheocast-Gußblöcke, wobei die Metallegierung eine kugelförmige mikrographische Struktur aufweist;
- dem Teilen dieser Rheocast-Gußblöcke in eine Anzahl von Gußblöcken mit einem vorbestimmtem Gewicht, wobei diese Rheocast-Gußblöcke mechanisch geschnitten werden;
- dem Aufheizen dieser geschnittenen Gußblöcke bis auf eine Temperatur innerhalb des Verfestigungsbereichs dieser Metallegierung, um die eine kugelförmige Struktur aufweisende Metallegierung in einen pastösen Zustand umzuwandeln;
- dem sequentiellen Zuführen dieser Gußblöcke in die Einspritzkammer der Spritzgußmaschine; und
- dem Einspritzen dieser kugelförmig strukturierten Legierung, die auf diese Temperatur innerhalb des Verfestigungsbereichs der Legierung geheizt wird, in eine Kokille;
- dadurch gekennzeichnet, daß in Kombination:
(a) - dieses Gießen der Metallegierung in einem halbflüssigen Zustand durchgeführt wild, indem die geschmolzene Metallegierung beim Verfestigen und unter laminaren Strömungsbedingungen durch einen statischen Mischer geführt wird, um die flüssige Legierung gleichmäßig mit einer festen Phase zu vermischen, die sich von der flüssigen Legierung absondert, um eine zeitweilig stabile Fest-/Flüssigaufschwemmung am Ausgang des Mischers zu erzeugen;
(b) - dieses Schneiden des Rheocast-Gußblocks auf solch eine Weise durchgeführt wird; daß jeder geschnittene Gußblock mit einem vorbestimmten Gewicht das gleiche Gewicht wie die Komponente zum Gießen aufweist;
(c) - dieses Aufheizen dieser geschnittenen Gußblöcke auf eine Temperatur innerhalb des Verfestigungsbereichs dieser Metallegierung durchgeführt wird, indem jeder geschnittene Gußblock in das Innere eines jeweiligen rostfreien Edelstahlbehälters gelegt wird, und der Gußblock und der Container in einem vorgeheizten Ofen aufgeheizt werden.

2. Verfahren nach Anspruch 1, dadurch gekennzeichnet, daß diese Temperatur innerhalb des Verfestigungsbereichs dieser Legierung und die chemische Zusammensetzung dieser Legierung so ausgewählt werden daß diese kugelförmig strukturierte Legierung, die auf eine Temperatur innerhalb des Verfestigungsbereichs der Legierung aufgeheizt wird, im wesentlichen pseudoplastische rheologische Eigenschaften und eine Viskosität in ruhendem Zustand von ungefähr 10⁷ P annimmt.

3. Verfahren nach Anspruch 2, dadurch gekennzeichnet, daß während dieses Einspritzverfahrensschritts diese Metallegierung eine feste und eine flüssige Phase aufweist, wobei diese feste Phase mindestens 50 % des Volumens einnimmt.

4. Verfahren nach einem der vorherigen Ansprüche, dadurch gekennzeichnet, daß dieser Schmelzverfahrenschritt darin besteht, Aluminiumlegierungsbarren, die einen vorbestimmten Prozentanteil einer feinverteilten Keramikmaterialphase beinhalten, aufzuschmelzen und in einem Gefäßofen durchgeführt wild, der mit einer Mischvorrichtung ausgestattet ist.

5. Verfahren nach Anspruch 4, dadurch gekennzeichnet, daß diese Keramikphase aus Silikonkarbidteilchen besteht.

6. Verfahren zum Spritzgießen einer Aluminiumlegierung, das darin besteht, einen Gußblock, der durch das Gießen dieser Legierung in einem halbflüssigen Zustand erzeugt wird, um eine kugelförmige mikrographische Struktur in der Legierung zu erzeugen, auf eine Temperatur innerhalb des Verfestigungsbereichs der Legierung aufzuheizen, um so die Legierung auf einen hochviskosen, halbflüssigen Zustand zu reduzieren, und darin, nachfolgend einen mechanischen Druck auf den Gußblock auszuüben, dadurch gekennzeichnet, daß Kokillen verwendet werden, die einen Zulauf besitzen, dessen Dicke ungefähr 2 bis 2,5 mm beträgt; und daß eine Aluminiumlegierung verwendet wird, die eine gleichmäßig verteilte Keramikphase enthält.

## Revendications

1. Procédé pour la production de pièces moulées sous pression, en particulier de composants pour moteur à combustion interne en alliage léger, comprenant les étapes consistant à :
- amener en fusion un alliage métallique jusqu'à ce qu'il devienne entièrement liquide ;
- couler l'alliage métallique sous forme semi-liquide ;
- solidifier l'alliage métallique sous la forme semi-liquide en lingots Rheocast dans lequel l'alliage métallique présente une structure micrographique globulaire ;
- diviser les lingots Rheocast en un certain nombre de lingots de poids prédéterminé par découpage mécanique de ces lingots Rheocast ;
- chauffer les lingots découpés à une température dans la plage de solidification de l'alliage métallique pour convertir l'alliage métallique de structure globulaire sous la forme pâteuse ;
- alimenter les lingots un par un dans la chambre d'injection d'une machine à coulée sous pression ; et
- injecter l'alliage à structure globulaire, chauffé à la température de la plage de solidification de l'alliage, dans un moule ;
- caractérisé par le fait qu'en combinaison :
(a)- la coulée de l'alliage métallique dans la forme semi-liquide s'effectue en amenant l'alliage métallique en fusion tel quel solidifié et dans des conditions d'écoulement laminaire par un mélangeur statique pour le mélange de l'alliage liquide uniformément avec une phase solide qui se sépare de l'alliage liquide pour produire une suspension solide-liquide provisoirement stable à la sortie du mélangeur ;
(b)- ce découpage du lingot Rheocast s'effectue de façon que chaque lingot découpé d'un poids prédéterminé présente le même poids que le composant pour la coulée ;
(c)- le chauffage des lingots découpés jusqu'à une température à l'intérieur de la plage de solidification de l'alliage métallique s'effectue en plaçant chaque lingot découpé à l'intérieur d'un conteneur en acier inoxydable respectif et en chauffant le lingot et le conteneur dans un four de préchauffage.

2. Procédé selon la revendication 1, caractérisé par le fait que la température à l'intérieur de la plage de solidification de l'alliage et la composition chimique de cet alliage sont sélectionnées de telle sorte que l'alliage à structure globulaire chauffé à une température dans la plage de solidification de l'alliage adopte des caractéristiques sensiblement rhéologiques pseudoplastiques et une viscosité au repos d'environ 10⁷ P.

3. Procédé selon la revendication 2, caractérisé par le fait que pendant l'étape d'injection, l'alliage métallique comprend une phase solide et une phase liquide ; la phase solide étant égale à au moins 50 % en volume.

4. Procédé selon l'une quelconque des revendications précédentes, caractérisé par le fait que l'étape de fusion consiste à porter en fusion de la fonte brute d'alliage d'aluminium contenant un pourcentage prédéterminé d'une phase de matériau céramique finement dispersé et est conduite dans un four pot équipé de moyens de mélange.

5. Procédé selon la revendication 4, caractérisé par le fait que la phase céramique consiste en particules de carbure de silicium.

6. Procédé pour le moulage sous pression d'alliage d'aluminium consistant à chauffer un lingot produit par coulée de l'alliage sous forme semi-liquide pour produire une structure micrographique globulaire de l'alliage à une température dans la plage de solidification de l'alliage et de façon à réduire l'alliage à une forme semi-liquide fortement visqueuse et ensuite à exercer une pression mécanique sur le lingot, caractérisé par le fait qu'il met en oeuvre des moules ayant une entrée dont l'épaisseur est d'environ 2 ö 2,5 mm ; et par le fait qu'il met en oeuvre un alliage d'aluminium contenant une phase de matériau céramique uniformément dispersée.
